

J. H. L. DE BATS,  
METHOD OF CARBONIZING IRON AND STEEL,  
APPLICATION FILED AUG. 19, 1918.

1,335,094.

Patented Mar. 30, 1920.

FIG.1.



FIG.2.



FIG.3.



WITNESSES

J. Herbert Bradley

INVENTOR

Jean Hubert Louis De Bats  
By Fredk. W. Winton  
Attorney

# UNITED STATES PATENT OFFICE.

JEAN HUBERT LOUIS DE BATS, OF ZELIENOPLE, PENNSYLVANIA, ASSIGNOR TO NEW PROCESS METALS CORPORATION, OF WILMINGTON, DELAWARE, A CORPORATION OF DELAWARE.

## METHOD OF CARBONIZING IRON AND STEEL.

1,335,094.

Specification of Letters Patent. Patented Mar. 30, 1920.

Application filed August 19, 1918. Serial No. 250,462.

To all whom it may concern:

Be it known that I, JEAN HUBERT LOUIS DE BATS, a resident of Zelienople, in the county of Butler and State of Pennsylvania, have invented a new and useful Improvement in Methods of Carbonizing Iron and Steel, of which the following is a specification.

This invention relates to a method of carbonizing iron and steel articles, and its object is to provide a method which will produce a substantially uniform carbonization of the article throughout its entire cross sectional area, and whereby the degree of carbonization can be controlled so as to produce substantially equal carbonization of a number of iron or steel pieces, thereby adapting the process to the production of tool steel stock and similar uses.

According to the usual methods of carbonizing iron and steel articles, said articles are packed in charcoal or other carbonizing material in a closed container which container is placed in a suitable heating furnace where its temperature is raised and this causes the carbon gases from the carbonizing material to penetrate and deposit carbon in the metal articles. With these old methods the penetration of the carbon into the article is limited, so that only a surface hardening is secured, or in case the carbonizing heat is continued so as to penetrate to or toward the center of the article, the amount of carbon in and near the outer surface of the article is much greater than that at or toward the center, and tends to become graphitic. Furthermore, when carbonizing small articles or pieces, a number are packed in the carbonizing material in the container, so that those nearest the exterior receive the greatest degree of heat and are carbonized to a greater degree than those near the center of the container.

With my method the above objections are overcome. In carrying out the method the articles or pieces to be carbonized, such for instance, as low carbon or soft steel, are preliminarily heated in any suitable way or in any suitable furnace to a point where the metal begins to become porous. Generally this condition is reached at a temperature of approximately 1100° centigrade. The pre-heating must be at a slow heat and continued for a sufficient length of time to insure the metal becoming porous throughout

the cross section of the article or piece. The pre-heated articles are then allowed to cool, either wholly or at least to below the point where they can ignite the carbonizing material, and are packed in suitable carbonizing material, preferably graphite, and preferably what is known as graphite "float," that is, graphite in a very fine condition, and are then subjected to the carbonizing process, either in the usual way as heretofore practised, but preferably in a rotary drum, to which heat is applied and which is rotated during this part of the process so as to subject all of the articles or pieces in the drum to substantially the same temperature and receive the same degree of carbon penetration. A suitable apparatus for this purpose is shown in the accompanying drawings, in which Figure 1 is a longitudinal section through the apparatus; and Figs. 2 and 3 are transverse sections showing respectively the condition in the drum when the latter is stationary and when it is rotating.

This apparatus comprises a drum 1 having heads 2 closing its ends and being provided with a refractory lining 3, such as refractory brick, backed by a heat insulating layer 4. This drum is provided with bands 5 and is mounted upon two sets of rolls 6, which contact with said bands and which are secured to the shafts 7, one, or both, of which is positively driven from any suitable source, such as by the belt pulley 8 secured to one of said shafts. The drum is rotated either by frictional contact of the rolls 6 with the bands 5, or, if desired, one or more of said rolls and bands may be toothed so as to secure a more positive drive. The drum is provided with an interior longitudinal heating flue or flues, preferably with a central flue as shown at 9. One end of this flue is suitably connected to a source of heat, such as a gas burner 10, projecting its flame into said flue, and its opposite end is connected by any suitable rotatable joint to a stack or chimney 11. The construction of this drum is specifically described and is claimed in my application of even date herewith, Serial No. 250,463.

The articles to be treated, shown at 12 (in this case tool steel stock or bars) together with the carbonizing material are placed in the drum, through a suitable door or doors indicated at 14, in one of the heads 110

of the drum. The annular space in the drum is only partially filled with such articles and carbonizing material, as shown in Fig. 2, so that during the carbonizing process the articles and the carbonizing material move around with the drum, as shown in Fig. 3. Since the drum rotates continuously and the articles move around therein, all of the articles or pieces are subjected to the same degree of heat, and the same degree of carbonization is effected. The temperature applied to the drum is substantially the same used in all carbonizing processes, from 800 to 850 degrees centigrade.

15 By first pre-heating the articles above the critical point, as heretofore pointed out, the molecules are opened so that when the articles are subjected to the action of the carbonizing material, which preferably will be graphite "float," the carbon gases penetrate into the article or piece, entirely to its center, and to substantially a uniform degree throughout the cross section of the article or piece.

25 It has been demonstrated that with this method soft steel, rods, bars or wires, such as used in the manufacture of nails, bolts, or the like, can be carbonized to possess an exceedingly fine, silky structure throughout 30 and such that the material is admirably adapted for cold chisels and other tools, thereby enabling the production of tool steel stock in a much cheaper and more expeditious manner than under prior practices.

35 Heretofore it has not been found feasible by carbonizing processes to produce tool steel stock, due to the fact that the penetration of the carbon is substantially only a surface one. Heretofore tool steels have been made 40 by melting in an open hearth, crucible, or electric furnace, a mixture containing the desired amount of carbon, pouring this to form an ingot, and afterward rolling, or forging down the ingot into the tool stock. On ac-

count of the hardness of the steel the rolling and forging is difficult, and such steels are, therefore, quite expensive. With, my method such tool steel can be produced much cheaper, by rolling, forging, or drawing down the soft steel to the desired cross section or shape, then pre-heating and carbonizing as above described, and insuring tool steel of uniform hardness and carbon content throughout and of a quality equal, if not superior, to the best quality of carbon tool steel manufactured according to the old processes.

What I claim is:

1. The herein described method of carbonizing iron and steel pieces consisting in preliminarily heating the pieces to a temperature of approximately 1100° centigrade, thereby causing the metal to become porous, cooling the same, and then subjecting the same to a carbonizing temperature while packed in carbonizing material.

2. The herein described method of carbonizing iron and steel pieces, consisting in preliminarily heating the pieces to a temperature of approximately 1100° centigrade, thereby causing the pores to open up, cooling the same, then subjecting the same, when associated with a carbonizing material, and when moving, to a carbonizing temperature.

3. The herein described method of carbonizing iron and steel pieces, consisting in preliminarily heating the pieces to a temperature of approximately 1100° centigrade, thereby causing the pores to open up, cooling the same, then packing in "float" graphite, then agitating, and simultaneously subjecting same to a carbonizing temperature.

In testimony whereof, I have hereunto set my hand.

JEAN HUBERT LOUIS DE BATS.

Witness:

G. G. TRILL.